# EUROPEAN PATENT SPECIFICATION

(11) **EP 0 125 752 B1**
(45) Date of publication and mention of the grant of the patent: **06.12.1989**
(21) Application number: 84301453.1
(22) Date of filing: 06.03.1984
(51) Int. Cl.: H01F 1/08

(54) **Bonded rare earth-iron magnets**
Gebundene seltene Erden-Eisen-Magnete
Aimants comportant des particules du système terre rare-fer et un liant

(30) Priority: 09.05.1983 US 492629
(43) Date of publication of application: 21.11.1984
(73) Proprietor: GENERAL MOTORS CORPORATION, Detroit Michigan 48202 (US)
(72) Inventor: Lee, Robert Weir, Troy Michigan 48084 (US); Croat, John Joseph, Sterling Heights Michigan 48077 (US)
(74) Representative: Haines, Arthur Donald

(56) References cited:
- EP-A- 0 066 348
- GB-A- 455 806
- GB-A- 1 190 636
- JP-A-57 141 901
- US-A- 4 197 146
- PATENTS ABSTRACTS OF JAPAN, vol. 6, no. 128 (E-118)[1006], 14th July 1982; & JP-A-57 54 304

## Description

This invention relates to a bonded particle permanent magnets and to a method of making them. In accordance with the invention, such magnets are readily fabricated into desired shapes from melt-spun rear earth-iron alloy ribbons. These magnets have intrinisic coercivities and energy products of the same order as samarium-cobalt magnets but are much less costly. The bonded magnet compacts are magnetically isotropic. They may be readily magnetized in any prefered direction in a suitable magnetic field.

### Background

There has long been a need for relatively inexpensive but very strong permanent magnets. Therefore, considerable work has been done on the development of alloys and processes for making magnets of exceptional strength.

Before this invention, sintered or bonded samarium-cobalt (Sm-Co) powder magnets have been used in applications where high magnetic remanence and coercivity are needed in a shaped permanent magnet. However, such Sm-Co power magnets are very expensive. The high price is a function of both the cost of the metals and the cost of their manufacture into magnets. Samarium is one of the least abundant rare earth elements, while cobalt is a critical metal with unreliable worldwide availability.

Processing Sm-Co powder magnets involves many critical steps. One such step is grinding alloy ingot into very find powder. Ideally, each powder particle is a single crystal that is inherently magnetically anistropic. To obtain an oriented permanent magnet, the anisotropic powder particles must be oriented in a magnetic field before the position of each particle is fixed by sintering or bonding. After sintering or bonding, the magnet must be finally magnetically aligned in the same direction in which the particles were intially oriented to obtain optimum magnetic properties. That is, the magnets are anisotropic. Sintered Sm-Co magnets may approach densities nearing 100% of alloy density. For bonded Sm-Co magnets, however, it is difficult to obtain densites much greater than about 75%. Conventional powder metal compaction equipment is not capable of achieving higher packing densities because of the shape and hardness of the powder particles.

This invention relates to high density, bonded, rare earth-transition metal magnets with properties nearly rivalling bonded samarium cobalt magents. However, these novel magnets are based on the relatively common and inexpensive light rare earth elements, neodymium and praseodymium; the trasition metal element, iron; and boron. These alloys and the method by which they are processed to achieve superior hard magnetic properties are described in detail in copending European application number 83304909.1.

For use in this invention, the magnetic alloys are made by melt-spinning. Melt-spinning is a process by which a molten stream of alloy is impinged on the perimeter of a rotating quench wheel to produce radidly quenched alloy ribbons. These ribbons are relatively brittle and have a very finely crystalline microstructure. They may be compacted and bonded as will be described herafter to create novel, isotropic, high density, high performance permanent magnets.

In JP-A-57 141901 a bonded magnet containing a permament magnet powder of amorphous alloy containing one or more transition metals, one or more elements of the group B, Si, P or C and rare earths elements is described. Magnetic energy products of 4.8 MGoe have been achieved.

In the following and

### Brief Summary

In accordance with a preferred practice of the subject invention, isotropic, bonded particle magnets are produced with compact densities of at least about 75% of the constituent RE-Fe alloy density. Unexpectedly, the constituent alloy does not have to be ground into a fine powder in order to obtain a magnet with high magnetic remanence. Rather, melt-spun rare rare earth-iron ribbon is simply compacted in a powder metal die in a suitable press.

At compaction pressures of about 1,103, 162 kPa (160,000 psi), a compact with a density of about 80% is achieved. The melt-spun ribbons facture during compaction into brick-like segments, each containing many randomly oriented crystallites. These segments pack together very closely, promoting both high compact density and green strength. The green compacts can be easily handled without damage. On the other hand, it has been found that compacting spherical powder particles of like alloy will not yield a green compact with any appreciable green strength. The compacts are so weak they cannot be removed from a die without fracture.

A preferred alloy for use herein would be a melt-spun form of Ndo.15(Feo.95Bo.c)5)0.as alloy having a suitable finely crystalline microstructure. The ribbon itself is magnetically isotropic. It need not be magnetized before or during compaction.

After pressing, the ribbon particles of the green compact are coated with a binder agent which may be later hardened to form a self-supporting, unmagenitzied but magentizable, magnetically isotropic, composite body. The binder agent may be a hardenable resinous substance such as an epoxy; a lower melting metal such as lead-tin solder; and any other suitable organic or inorganic binder.

By practicing this invention, one can now make a megntizable body of bonded melt-spun alloy ribbons in almost any desired shape. The ribbon segments may be compacted to high density in almost any conventional die press. Furthermore, the compacts are magnetically isotropic. This is, they may be magnetized in any desired direction to achieve optimum properties for a particular application.

For example, arcuate shaped field mangets for direct current motors could be formed by compacting melt-spun rare earth-iron ribbon in a punch and die set. These arcuate shaped bodies would first be magnetized after compaction in an applied magnetic field in which the field lines radially intersect the compact to incude radially oriented, remanent magnetization. In like manner, a bonded magnet of any other shape could be magnetized in a magnetic field having field lines oriented in any desired direction.

The invention will be better understood in view of the Figures and detailed description which follow.

Figures
Figures 1(a) to 1(d) are schematic illustrations of the manufacture of a right circular cyclindrical shaped magnet in accordance with the invention.
Figure 2 is a second quadrant demagnetization plot for a bonded magnet made in accordance with the invention compared to the demagnetization of an unbonded sample of melt-spun ribbons of the same rare earth-iron alloy normalized to 100% density.
Figure 3 is a plot of compaction density as a function of uniaxial compaction pressure for a right circular cyclindrical magnet body formed of melt-spun rare-earth ribbon.
Figure 4 is a plot comparing second quadrant demagnetization for oriented Sm₂Co_{"} and SmCo₅ bonded powder magnets and melt-spun bonded Nd-Fe-B powder magnets.
Figures 5 and 6 are scanning electron micrographs of cut and polished sections of compacted and epoxy bonded magnets of melt-spun Nd-Fe-B alloy ribbon.

### Detailed Description and Examples

In accordance with a preferred embodiment of the invention, iron, rare earth elements and a small amount of boron are melted and rapidly quenched by the melt spinning process to create relatively brittle alloy ribbons. These alloys have high inherent intrinsic coercivities of the order of a kilooersted or more, some higher than twenty kiloOersteds and remanent magnetization of the order of 8 kiloGauss. Such high coercivities and high remananet magnetism are believed to be due to the pressure of a very finely crystalline phase (atomic ordering less than about 500 nanometers) composed of iron and low atomic weight rare earth elements (atomic No. less than or equal to 62) that do not have full or exactly half full f-orbitals. The phase is stablized by the presence of a small amount of boron. European application No. 83304909.1 describes suitable compositions and methods of making such and is incorporated herein by reference.

Preferred alloys contain from about 10 to 50 atomic percent neodymium, praseodymium; or mischmetal comprised principally of these rare earth elements; a small amount of boron (generally less than about 10 atomic percent); and the balance iron. Other rare earth elements such as samarium and transition metal elements such as cobalt may be incorporated in amounts that do not severely degrade the magnetic properties of the melt-spun alloys. Other metals may be incorporated in small amounts which tend to dilute but not destroy the magnetic properties of the preferred melt-spun RE-Fe alloys.

A preferred method of making the high coercivity alloys is to melt suitable amounts of the elements together and then quench a stream of the alloy on the permiter of a spinning quench wheel to create a friable alloy ribbon with a very finely crstalline microstructure. This process is referred to herein as melt-spinning.

Figure 1 is a schematic representation of a method for making bonded permanent magnets in accordance with the invention. Referring to Figure 1 (a), the alloy 2 is melted in a crucible 4 and ejected through a small orifice 6. The ejected stream of alloy impinges on a rotating quency wheel 8 to form a ribbon 10·of solidified alloy with a very finely crystalline phase. Ribbon 10 is generally quite thin and very brittle. It can be broken into pieces small enough to fit into a die cavity by almost any crushing means. Melt-spun ribbons have been placed, for example, between two clean sheets of paper and an ordinary wooden writing pencil has been rolled over the sandwiched material. The resultant ribbon segments can be poured directly into a die cavity. Ball-milling or otherwise milling the ribbon in air creates smaller ribbon sections but does not cause any detectable loss of magentic properties or compactability in conventional tooling. It has been noted, however, that some deterioration of magnetic properties occurs when ribbons are ground for excessively long periods of time.

Figure 1 (b) shows a die for making a cylindrical compact 12. The compact is formed between a pair of opposing punches 14 and 16 in tool 18. This process is referred to herein as uniaxial compaction, the axis being parallel to the travel of the compaction punches. It has been found that under ordinary conditions for making conventional powder metal compacts of iron or other such metal powders, rare earth-iron compacts of eighty percent density or greater can be made. The compacting process apparently tends to fracture the subject RE-Fe ribbon segments and to pack them together in a manner such that the ribbon sections lie parallel and directly adjacent to each other almost as the bricks in a brick wall are oriented with respect to one another. Each ribbon segment is much larger than a single magnetic domain. It is magnetically isotropic and is readily magnetized to a strong permanent magnet in an applied magnetic field.

As shown at Figure 1 (c), once a desired compact density is achieved, compact 12 is removed from the press and placed in side-arm tube 20. A hardenable liquid resin 22 is retained in a syringe 24. Syringe needle 26 is inserted through stopper 28 and a vacuum is drawn through the side arm of tube 20. Once tube 20 is evacuated, enough resin 22 is dripped onto compact 12 to saturate the pores between particles. The resin is then cured and any excess is machined away.

This bonded body 30 need not be magnetized when it is formed. Permanent magnetism is induced in the bonded compact body 30 by exposing it to a magnetic field of suitable direction and field strength. The field may be created by suitable magnetizing means such as a magentic induction coil 32. Coil 32 is activated to create a field represented by flux lines 34. The flux lines 34 run parallel to the axis of the cylindrical bonded body 30.

Clearly, in accordance with this invention, magnets can be formed in almost any shape that is adaptable to formation by powder metal pressing techniques such as uniaxial compaction in a rigid die or isostatic compaction in a flexible sleeve. A key advantage of this method over the conventional methods of making particulate Sm-Co magnets is that the compaction need not take place concurrently with magentization. Nor do the ribbons have to be ground to a size commensurate with single domain size. The rare earth-iron alloy ribbon of this invention is isotropic and need not be magnetized until after the bonded magnet is fully formed. This simplifies the magnet making process and eliminates all the problems associated with grinding fine powders and handling magnetized green compacts. Unexpectedly high remnant magnetizations of 7 kiloGauss (at least 6 kiloGauss being desired) and energy products of 9 megaGauss Oersted or more have been achieved.

How the quenched alloy particles are coated or impregnated to effect binding is not critical to this invention. While the preferred practice, to date, employs hardenable liquid epoxy binder resin, any other type of polymeric resin that does not interfere with the magnetic properties of the rare earth-iron alloys would be suitable. In fact, almost any type of organic or inorganic binder may be used so long as it does not adversely effect the magnetic properties of the alloys.

For example, a very thin layer of lead or other low melting metal could be sputtered or sprayed on to melt-spun alloy ribbon before compacting. The compact could then be heated to melt the lead and bond the particles. Another practice would be to blend melt-spun RE-Fe ribbon fragments with a dry resin powder. After compaction, the resin would be cured or melted at a suitable elevated temperature to bond the alloy particles.

It is only necessary to achieve adequate bonding strength to stabilize the motion of the constituent alloy particles for whatever application in which the magnet body is to be used. In some cases, a wax binder would be sufficient; in others, a relatively rugged and highly adhesive binder such as an epoxy would be more advantageous.

Another clear advantage of the invention is that the direction of magnetization of the bonded rare earth iron body can be tailored to a desired application. The body is first magnetized afer it is shaped and the alloy particles are mechanically bonded together. Thus, the unmagnetized body is simply placed in magnetic field of desired direction and adequate strength to establish its remanent magnetic direction and energy product. The magnet bodies can be made and stored in an unmagnetized state and be magnetized immediately before use. A preferred practice would be to install a bonded compact in the device in which it will be used and only then magnetize it in situ.

The neodymium-iron alloys of the following examples were all made by melt spinning. The melt spinning tube was made of quartz and measured about 102 mm (4 inches) long and 12.7 mm (Y₂ inch) in diameter. About 5 grams of premelted and solidified mixtures of pure neodymium, iron and boron metals were melt-spun during each run. The mixtures were remelted in the quartz tube by means of an induction coil surrounding it. An ejection pressure of about 34.47 kPa (5 psi) was generated in the tube with argon gas. The ejection orifice was round and about 500 urn in diameter. The orifice was located about 3.18 mm to 6.35 mm (½ to % inches) from the chill surface of the cooling disc. The disc was rotated at a constant revolution rate such that the velocity of a point on the perimeter of the disc was about 15 meters per second. The chill disc was orginally at room temperature and was not externally cooled. The resultant melt spun ribbons were about 30-50 pm thick and about 1.5 millimeters wide. They were brittle and easily broken into small pieces. Melt spun ribbons processed in this manner exhibited optimum magnetic properties for a given RE-Fe-B composition.

### Example 1

A 15 gram sample of melt-spun Nd_{0,2}(Fe_{0.95}B_{0.05})_{0.8} ribbon was ground in an argon atmosphere in a vibrating mill (Shatterbox, Spex Industries). The resultant powder was sieved to a particle size less than about 45 pm.

The powder was then placed in a rubber tube with an internal diameter of 8 mm. Rubber plugs sized to be slidable within the tube were inserted in either end. Steel rams were then inserted in either end of the tube. This assembly was placed in a pulsed magnetizing coil having a field strength of 40 kOe. The field was pulsed, drawing the rams together and causing the plugs to compress and lightly compact the powder between them. If the powder particles were magnetically ansiotropic, this pulsed pressing step would physically orient them along their individual preferred magnetic axes.

The rams were removed from the tube and the excess rubber sleeve was trimmed away. The plugged tube was then reinserted into a hydraulic press and compacted between rams to a pressure of 1,103,162 kPa (160,000 pounds per square inch).

The resultant right circular cylindrical compact measured 8 mm high and 8 mm diameter. The compact could be handled without breaking. It was taken out of the rubber compaction tube and placed in a side arm Pyrex test tube. The tube was evacuated with a mechanical vacuum pump. A hypodermic needle attached to a syringe carrying liquid epoxy resin was then inserted through the rubber stopper of the tube. The resin was dropped into the tube to saturate the compact. The epoxy was a conventional commerically available epoxy comprised of a diglycidyl ether of bisphenol-A diluted with butyl glycidyl ether and cured with 2-ethyl-4-methyl-imidazole. The compact was removed and allowed to cure overnight (approximately 16 hours) in air at 100°C).

It was magnetized in the direction of precompaction, i.e. parallel with the original pulsed magentic field, with a 40 kilooersted pulsed magnetic field. This was the maximum magnetic field available at the time. The field is believed to be too weak to reach magnetic saturation of the RE-Fe-(3 alloys. Therefore, stronger fields might produce even stronger magnets. The room temperature demagnetization (second quadrant) plot of the hysteresis curve of this bonded magnet composition is shown in Figure 2. Magnetic measurements were made on a vibrating sample magnetometer, Princeton Applied Research (PAR) Model 155, at a room temperature of about 25°C. The sample was a cube about 2 mm on a side machined from the cylindrical magnet to fix in the magnetomoter sample holder.

Figure 2 compares demagnetization curves for non-bonded powder of the same melt-spun ribbon batch as those used for the compact, corrected to 100% density (i.e., density of the alloy). The density of the alloy ribbon in the compact was 85% of the density of the alloy itself as determined by standard density measurement in water. The bonded magnet formed from the 85% dense compact has a residual magnetic indication of 85% of that of the unbonded melt spun ribbon corrected to 100% density.

### Example 2

An experiment was run to determine the difference between (1) a bonded magnet in which the finely ground alloy (less than 45 pm) ribbon particles were concurrently magnetically aligned and prepressed in a pulsed magneticfield, and (2) a bonded magnet formed from unaligned ground alloy particles. Powder particles of the same size and composition as the melt-spun ribbon of Example 1 were precompacted in a plugged rubber sleeve in a hand press but without current application of a magnetic field. The excess rubber at the ends of the sleeves was trimmed away and reinserted in a tool in the hydraulic press. The powder preform was finally compacted at a pressure of about 1,103,162 kPa (160 kpsi). The resultant 8 mm thick compact was then fabricated in every other respect identically to the preoriented magnet of Example 1. The demagnetization curve for the unaligned bonded magnet was identical to that of the prealigned magnet plotted in Figure 2.

This experiment illustrates the magnetically isotropic behaviour of the melt-spun, rapidly quenched alloy particles. The sieved powder included all particle fractions smaller than 45 micron metres, with many particles smaller than one micrometer, to align. If the smallest particles were near enough single domain size they would be expected to align along the field lines during the alignment step of Example 1. When so aligned and magnetized in the same direction, the resultant magnets should have measurably higher residual induction and a more square hysteresis loop than unoriented magnet counterparts if the method had achieved near domain size, magnetically anisotropic alloy particles. Thus, while the very finely crystalline alloys may be made up of very tiny crystallites which would be expected to have preferred axes of magnetic alignment, apparently, they cannot be ground finely enough by ball milling to take advantage of magnetic alignments during the pressing step. It is not believed that using other state-of-the-art milling techniques would provide different results so far as the creation of near domain size, anisotropic particles from the subject melt-spun alloys is concerned.

Another proof of the isotropic nature of the ribbon particles was made as follows. The pre- pulsed and compacted bonded magnet sample (2 x 2 mm cube) of Example 1 was demagnetized. The sample was then pulsed in a 40 kOe field in a direction transverse to the original direction of magnetic alignment. The demagnetized curve for the sample magnetized in the transverse direction was then taken. It was exactly the same as the demagnetization curve taken for the original alignment direction (shown in Figure 2). Because the demagnetization curves were the same for magnetization in the direction of alignment during compaction and for demagnetization transverse thereto, it must be concluded that there was not magnetic alignment of particles in the pulsed precompaction.

That is, the ground powders and bonded compacts are both magnetically isotropic.

### Example 3

A comparison was made between isostatically and uniaxially pressed magnets made from unground dₒ,_{Z}(Feₒ,_{sS}Bₒ.ₐₛ)ₒ.ₑ alloy ribbon particles. The ribbons initially had a cross-section of approximately 2 mm (width) by 30 urn (thicknes). The alloy ribbon as melt-spun was easily fractured into small pieces preparatory to compaction. The relationship of compact density to uniaxially applied pressure for fractured Nd-Fe-B ribbon particles pressed in the direction of the axis of a right circular cylindrical compact is shown in Figure 3. The compaction curve becomes flatter above about 1,103,162 kPa (160,000 pounds per square inch) at a density of approximately 83 percent (6.24 grame per cm³) of the ribbon density (7.35 grams per cm³).

Figures 5 and 6 are scanning electron micrographs of isostatically compacted, epoxy bonded magnets made in accordance with this example. In the micrographs, the lighter regions are Nd-Fe-B melt-spun ribbon while the dark regions are epoxy resin or voids. The white line in the lower right-hand corner of each micrograph represents a length of 100 pm. Both are plan views of a section of isostatically pressed melt-spun ribbon that was not ground prior to compaction. The ribbon segments each contain many crystallites.

It is clear for Figures 5 and 6 that the melt-spun ribbon fractures and compacts in a manner such that individual ribbon segments line up with their long edges substantially parallel to one another. The flat planes of the particles lie facing one another with very little space therebetween. This probably accounts for the high compaction densities. It has been found that, by disposing a sample in an elastic tube, stopping the ends, and isostatically exerting a pressure of 1.103,162 kPa (160,000 pounds per square inch), a compact density of 87% (6.55 grams per cm³) is achieved. The arrangment of the relatively large ribbon segments also seems to provide the high density compacts with good green strength. This with reasonable care they can be handled prior to bonding without breaking or chipping.

Spherical powder particles of a like alloy do not compact well under like conditions. The green compacts are so weak that they cannot be handled prior to bonding.

Figure 5 especially points out that there are several different regions of ribbon segments oriented parallel to one another in each compact. For example, the particles in the region labeled 50 are oriented at an actue angle with respect to the particles in the region labelled 52.

Figure 6 shows an enlarged section of a compact where the close packing arrangement of the ribbon segments to one another is clearly visible.

Thus, it has been unexpectedly found that melt-spun ribbons of rare earth-iron alloys are relatively easy to compact to densities over 80 percent employing ordinary uniaxial or isostatic pressing means. The compacts have very high green strengths. It has also been found that there is no apparent advantage in pre-milling the alloy compositions. In fact, over-milling ribbon samples was found to adversely affect the magnetic properties of the material, i.e., reduce the remanent magnetization and energy product of magnets made from the over-milled materials.

It has also been found that the use of conventional die and powder metal lubricants such as powdered boron nitride does not either adversely or positively affect the compact. However, in practice such libricants may be desirable to minimize die wear.

Figure 4 qualitatively compares the second quadrant hysteresis of the bonded Nd-Fe-B magnets of the preceding examples with bonded and magnetically prealigned Sm₂C₀₁₇ and (Sm, mischmetal) Co₅ magnets. Oriented Sm₂Co₁₇ magnets made from near domain size powder particles, magnetically aligned during compaction, sintered, heat-treated and then finally magnetized exhibit the highest remanent magnetization, Bᵣ of approximately 11 kiloGauss. Sintered oriented Sm-Coₛ magnets (substantially 100% density) have a Bᵣ of approximately 8.5 kiloGauss.

The unoriented Nd-Fe-B magnets of this invention fail about midway between the prealigned and bonded Sm2Co" type and the SmCoₛ type magnets. Our magnets are far superior to unaligned bonded Sm-Co magnets.

Oriented ferrite magnets have much lower remanent magnetization than the bonded magnets of the present invention and Alnico magnets have much lower coercitivities. Given the tremendous cost and processing advantages of the magnets of the present invention, the fact that they approach the magnetic strength of the best oriented rare earth-cobalt magnets makes them highly commercially adaptable.

The strength of the magnets of the present invention is obviously a function of the quality, i.e., the intrinsic magnetic properties of the constituent melt-spun rare earth-iron alloy. Melt-spun alloys with higher coercivities and remanent magnetization values would produce even stronger hard magnets than those disclosed herein.

In conclusion, novel bonded magnets have been produced from fractured and compacted melt-spun rare earth-iron alloy ribbons. The magnets are magnetically isotropic. They do not have to be magnetically prealigned yet they have properties rivalling those of much more expensive bonded samarium cobalt magnets.

The method of the present invention may be used to make cylindrical magnets, arcuate- shaped magnets, irregularly shaped magnets, square magnets, and magnets of almost any shape which can be formed by powder metal compaction methods. Never before has it been possible to efficiently and inexpensively produce such high quality permanent magnets of such varying shape from relatively inexpensive starting materials.

While the invention has been described in terms of specific embodiments thereof, other forms may be readily adapted by one skilled in the art. Accordingly, the invention is to be limited only by the following claims.

## Claims

1. A permanent bonded magnet (30) formed of melt-spun alloy ribbon particles that have a very finely crystalline magnet phase, said alloy comprising one or more rare earth elements taken from the group consiting of neodymium, praseodymium, and mischmetals; the transition metal element, iron; and boron; the particles in said magnet are maintained in a desired magnet shape (12) by a binding agent (22) interdispersed therebetween; and the particles are magnetically isotropic and the magnet shape (12) may be magnetized in any desired direction in a suitable magnetic field (34) to form the bonded magnet (30) with a particle compact density of at least 80% of the alloy density, characterized in that said magnetic bonded magnet has a magnetic energy product of at least nine megaGauss Oersted at magnetic saturation.

2. A permanent bonded magnet (30) according to claim 1, with particles of a friable, rapidly quenched, finely crystalline, melt-spun alloy ribbon (10), and said particles are fractured and compacted under pressure into a compact (12) with said magnet shape, in a die having the shape of said magnet, said fractured and compacted particles in the compact (12) then being fixed in said magnet shape by said binding agent (22); and said compact (12) being equally susceptible to magnetization in any desired direction in the presence of a magnetic field of suitable direction and magnitude to form a permanent magnet (30).

3. A permanent bonded magnet (30) according to claim 2, with said particles having a substantially brick-like shape and being spacially oriented substantially parallel to each other within regions of the compact (12) to achieve high compact densities and compact green strength; said compact (12) being equally susceptible to magnetization in any direction in an applied magnetic field of suitable strength and direction such that at a compact density of 80% of said alloy the magnet (30) formed has a magnetic remanence of at least six kiloGauss (0,6 T).

4. A permanent bonded magnet (30) according to claim 2 or 3 with said particles each consisting of a plurality of individual fine crystals.

## Patentansprüche

1. Gebundener Permanentmagnet (30) aus schmelz-gesponnenen Legierungsbandteilchen, die eine sehr feinkristalline Magnetphase besitzen, wobei die Legierung enthält ein Seltenerd-Element oder mehrere Seltenerd-Element aus der aus Neodym, Praseodym und Mischmetallen bestehended Gruppe; das Übergangsmetall-Element Eisen; und Bor; die Teilchen in dem Magnet in einer gewünschten Magnetform (12) durch ein dazwischen dispergiertes Bindemittel (22) gehalten sind; die Teilchen magnetisch isotrop sind und die Magnetform (12) in jeder gewünschten Richtung in einem geeigneten Magnetfeld (34) magnetisiert werden können, um den gebundenen Magneten (30) zu bilden mit einer Teilchenkompaktdichte von mindestens 80% der Dichte der Legierung, dadurch gekennzeichnet, daß der gebundene Magnet ein Magnetenergieprodukt von mindestens neun MegaGauss Oersted (71,64 kJ.m-³) bei magnetischer Sättigung besitzt.

2. Gebundener Permanentmagnet (30) nach Anspruch 1, mit Teilchen aus einem bröckligen, rasch abgeschreckten, feinkristallinen schmelz-gesponnenen Legierungsband (10), wobei die Teilchen gebrochen und unter Druck zu einer Kompaktform (12) mit der Magentgestalt kompaktiert sind in einer Form mit der Gestalt des Magneten, die gebrochenen und kompaktierten Teilchen in der Kompaktform (12) dann durch das Bindemittel (22) in der Magnetgestalt verfestigt sind; und die Kompaktfrom (12) gleichermaßen für Magnetisierung in einer gewünschten Richtung in Anwesenheit eines Magnetfeldes von geeigneter Richtung und Größe suszeptibel ist um eine Permanentmagneten zu bilden.

3. Gebundener Permanentmagnet (30) nach Anspruch 2, bei dem die Teilchen eine im wesentlichen quaderartige Form besitzen und räumlich im wesentlichen parallel zueinander innerhalb Bereichen der Kompaktform (12) orientiert sind, um hohe Kompaktform-Dichten un Kompatform-Rohfestigkeit zu erreichen; wobei die Kompaktform (12) in gleicher Weise für Magnetisierung in irgendeiner Richtung in einem angelegten Magnetfeld geeigneter Stärke und richtung suszeptibel ist, so daß eine Kompaktform-Dichte von 80% der Legierung des gebildeten Magneten (30) eine magnetische Remanenz von mindestens sechs kiloGauss (0,6 T) besitzt.

4. Gebundener Permanentmagnet (30) nach Anspruch 2 oder 3, bei dem die Teilchen jeweils aus einer Vielzahl von einzelnen feinen Kristallen bestehen.

## Revendications

1. Aimant permanent aggloméré (30) formé de particules d'un raban d'alliage filé à l'état fondu ayant une phase d'aimant très finement cristalline, l'alliage contenant un ou plusieurs éléments des terres rares choisis dans le groupe constitué par le néodyme, le praséodyme et les mischmé- taux, du fer comme métal de transition, et du bore, les particles de l'aimant étant maintenues à la configuration voulue (12) pour l'aimant par un agent liant (22) dispersé entre les particules, les particules étant magnétiquement isotropes et l'aimant formé (12) pouvant être aimanté dans n'importe quelle direction dans un champ magnétique convenable (34) pour former l'aimant aggloméré (30) avec une densité sous forme d'ébauche formée de particules qui est au moins égale à 80 % de la densité de l'alliage, caractérisé en ce que l'aimant aggloméré a un produit énergétique magnétique au moins égal à 71,64 kJ/m³ (9 MGOe) à la saturation magnétique.

2. Aimant permanent aggloméré (30) selon la revendication 1, ayant des particules d'un raban (10) d'alliage filé à l'état fondu, finement cristallin, friable et rapidement refroidi, les particules étant fracturées et comprimées sous pression sous forme d'une ébauche (12) ayant la configuration de l'aimant, dans un moule ayant la configuration de l'aimant, les particules fracturées et comprimées de l'ébauche (12) étant ensuite fixées à la configuration de l'aimant par l'agent liant (22), l'ébauche (12) pouvant subir une même aimantation dans n'importe quelle direction désirée en présence d'un champ magnétique de direction et d'amplitude convenables pour former un aimant permanent (30).

3. Aimant permanent aggoloméré (30) selon la revendication 2, dans lequel les particules ont une configuration analogue à celle de briques et sont orientées dans l'espace sensiblement parallèlement les unes aux autres dans des régions de l'èbauche (12) afin qu'elles donnent des ensités élevées d'ébauche et une résistance mécanique élevée de l'ébauche à l'étate cru, l'ébauche (12) pouvant être également aimantée dans n'importe quelle direction dans un champ magnétique appliqué ayant une intensité et une direction convenables afin que, pour une densité d'ébauche de 80% de celle de l'alliage, l'aimant formé (30) possède une aimantation rémanente d'au moins 0,6 T (6 kG).

4. Aimant permanent aggloméré (30) selon la revendication 2 ou 3, ayant des particules consistant chacune en un certain nombre de fins cristaux individuels.
